

Oct. 10, 1967

KARL-GEORG SPEITH ET AL 3,346,035  
PREVENTING THE OVERFLOW OF LIQUID METAL FROM AN END  
CASTING HEAD DISCHARGED IN A CURVED CONTINUOUS  
CASTING PATH TOWARDS THE HORIZONTAL PLANE  
Filed Feb. 18, 1965



Inventors:  
Karl-Georg Speith  
and Adolf Bungeroth,  
By *James A. Marwick*,  
Their Attorney.

1

2

3,346,035

**PREVENTING THE OVERFLOW OF LIQUID METAL  
FROM AN END CASTING HEAD DISCHARGED  
IN A CURVED CONTINUOUS CASTING PATH  
TOWARDS THE HORIZONTAL PLANE**

Karl-Georg Speith, Duisburg, and Adolf Bungeroth, Duisberg-Huckingen, Germany, assignors to Mannesmann Aktiengesellschaft, Dusseldorf, Germany, a corporation of Germany

Filed Feb. 18, 1965, Ser. No. 433,752  
Claims priority, application Germany, Feb. 20, 1964,  
M 59,992  
3 Claims. (Cl. 164—82)

The invention relates to continuous casting and relates more particularly to the continuous casting in a curved-discharge path of steel billets in which the descending billet is deflected to the horizontal plane and wherein during the normal casting operation the liquid sump projects with its leading point and a portion to the rear thereof to a minor and major extent into the horizontal plane.

During the continuous casting operation in the aforesaid manner, there exists the hazard that when the continuous casting operation comes to an end and the last piece of the casting in form of an end casting head descends out of the mold and gradually is transported into the horizontal position, liquid steel may spill or overflow or flow out of the end casting head; on this occasion, indeed, the entire remainder of the still liquid sump may be spilled through the opening of the end casting head, as soon as the end head of the billet enters into the horizontal. Such a spilling would, of course, have a core deteriorating effect.

Even if at the end of the casting operation a much reduced ferrostatic pressure enables the forming of billets without any deterioration in the core quality, this would presuppose that in the terminal end portion of the billet there is still maintained a mass head effect until the last liquid drop of steel has been solidified in the end head.

The aforesaid mass head effect operates in a core condensing manner from the beginning until the end of the casting operation, and remains effective for a while even after the teeming of molten steel into the mold has been halted, namely as long as liquid steel descends alone in the casting direction into the leading point of the sump which is formed by the converging solidification fronts.

In continuous curved casting with a horizontally positioned liquid sump end it is necessary that during idling of the machine no core deteriorating overflow occurs in end head of the billet.

It is accordingly among the principal objects of the invention to restrain during idling of the machine any overflow from the end head of the billet.

It is another object of the invention to provide for a curved-discharge technique with a reduced casting speed at least shortly before the termination of steel delivery or teeming into the mold.

It is still a further object of the invention to reduce the casting speed from the beginning of the end period of the casting operation.

It is yet another object of the invention to provide for reduction of the casting speed to such a degree that the leading point of the liquid sump will recede along the curved-discharge path of the billet to a position above and in advance of the horizontal plane.

With the above and other objects of the invention in view, the invention consists in the novel methods, construction, arrangement and combinations of various devices, elements and parts, as set forth in the claims hereof, one embodiment of the same being illustrated in the accompanying drawing and described in the specification.

In accordance with the invention, the aforesaid drawbacks attendant upon overflow can be avoided by reducing the casting speed at least shortly before steel delivery into the mold ceases. Reduction of the casting speed is preferred when the end period of the casting operation sets in. In any event the reduction of the casting speed should be sufficient so that the leading point of the liquid sump recedes along the discharge path to a position upstream of the horizontal plane.

In the appended drawing the single view is a schematic side elevational view, partly in section, of a billet during its curved-discharge path after the mold.

Reference is had to the following: "The Continuous Casting of Steel," by L. V. Gallagher and B. S. Old, *Scientific American* (December 1963), pp. 75-88.

Referring to the drawing, when the normal liquid sump stretch  $S_N$ , which equals 100 percent, during the casting operation is positioned with its leading point at  $x$  percent of the horizontal, its length before the end of the casting operation should be in good time reduced to the value  $S_E$  in accordance with the formula

$$S_E < S_N (100 - x) \text{ percent}$$

This is achieved by reducing the normal casting speed  $V_N = 100$  percent to  $V_E < V_N (100 - x)$  percent; wherein the leading point of the sump is caused to recede back to the desired position. This recession always needs a period of time which corresponds to the billet solidification time  $T$ . The pre-calculated reduction in casting speed must therefore be applied at the latest  $T$  minutes before the end of the billet solidification, or at the latest when the steel delivery to the mold stops.

*Example*

In casting a billet of an edge length of 200 x 200 mm. the casting speed  $V_N$  is assumed to be 900 mm./min. Under these conditions—at constant cooling—the length of the liquid sump  $S_N$  is 8 m.

In a curved-discharge casting machine the distance of the liquid sump of 8 m. is situated for a stretch of about 6 m. in the curved portion of the billet and the remainder which equals about 2 m. is disposed in the horizontal plane. Before the idling of the machine, the length of the sump should be diminished for more than 2 m.—for instance, for 2.5 m.—to about 5.5 m.

This is done by correspondingly reducing the speed  $V_N = 900$  mm./min. to the end speed  $V_E$  at the moment of discontinuing the casting operation:

$$\frac{V_E}{V_N} = \frac{S_E}{S_N}; \frac{V_E}{900} = \frac{5.5}{8.0}$$

$$V_E = 620 \text{ mm./min.}$$

At the instant of termination of the casting operation (at the end of steel feeding), the casting speed must be reduced to 620 mm./min. and continuing at a reduced withdrawal speed sufficiently long so that the leading sump point will recede in the horizontal towards the casting head in the casting curve and will coincide with the end head before the horizontal is reached.

We wish it to be understood that we do not desire to be limited to the exact details of construction shown

and described, for obvious modifications will occur to a person skilled in the art.

Having thus described the invention, what we claim as new and desired to be secured by Letters Patent, is as follows:

1. In a method of preventing the overflow of liquid metal from an end casting head of a casting discharged in a curved continuous discharge path towards the horizontal plane during the terminal period of the casting operation, the steps comprising, reducing the casting speed at least shortly before the end of the steel delivery to the mold to reduce the length of the sump and continuing withdrawal at a reduced casting speed so that thereafter the leading point of the sump is maintained above the horizontal.

2. In a method, as claimed in claim 1, the reduction of the casting speed commencing at the beginning of the terminal period of the casting operation.

3. In a method, as claimed in claim 2, the reduction of the casting speed being sufficient so that the leading point of the liquid sump which during the preceding normal casting operation was positioned at a point in the horizontal plane, will be forced to recede along the path to a position upstream of said point and above the horizontal plane.

#### References Cited

10      Continuous and Pressure Casting, published by Association of Iron and Steel Engineers, Pittsburgh, Pa., 1964, p. 14.

15      J. SPENCER OVERHOLSER, *Primary Examiner.*

          R. S. ANNEAR, *Assistant Examiner.*